

No. 660,426.

Patented Oct. 23, 1900.

S. GROSSIORD.

MANUFACTURE OF ARTIFICIAL STONES.

(No Model.)

(Application filed Oct. 6, 1898.)

FIG.1.



FIG.2.



FIG.3.



FIG.3<sup>bis</sup>



FIG.1<sup>bis</sup>



FIG.2<sup>bis</sup>



FIG.4.



FIG.5.



WITNESSES:

F. W. Wright  
S. C. Connor

INVENTOR

SAMUEL GROSSIORD

BY

Howson and Howson  
HIS ATTORNEYS.

# UNITED STATES PATENT OFFICE.

SAMUEL GROSSIORD, OF AUX MOUSSIERES, FRANCE.

## MANUFACTURE OF ARTIFICIAL STONES.

SPECIFICATION forming part of Letters Patent No. 660,426, dated October 23, 1900:

Application filed October 6, 1898. Serial No. 692,837. (No specimens.)

To all whom it may concern:

Be it known that I, SAMUEL GROSSIORD, lapidary, a citizen of the Republic of France, residing at Aux Moussieres, Jura, in the Republic of France, have invented certain new and useful Improvements in the Manufacture of Artificial Stones, of which the following is a specification.

This invention relates to improvements in the manufacture of artificial stones employed in jewelry.

The object of the invention is to impart to such stones if they are white imitations a scintillation resembling as nearly as possible that of a real diamond and if they are differently-colored imitations clearly-defined and distinct colorations.

The essential feature of my invention consists in welding a sheet or plate of window-glass between two blocks of the imitation products commonly termed "paste" and then cutting the block thus formed in the ordinary manner. On the same principle a white or colored block of the imitation material may be inserted between two plates of window-glass, or, in other words, the above process may be reversed. It is, moreover, possible to use but one single block of white or colored imitation material welded on a single plate of window-glass, which latter after the cutting forms either the base or the top of the stone.

In order that my invention may be thoroughly understood, I will describe the same with reference to the accompanying drawings, in which—

Figure 1 is a perspective view showing two blocks *a* and *b* of imitation material of one and the same quality and a sheet or plate *c* of window-glass adapted to be interposed between the two masses or blocks of imitation material. Fig. 1<sup>bis</sup> is a perspective view representing a block *a* of imitation material and two sheets or plates *c* and *c'* of window-glass, between which the said block *a* is to be interposed. These different pieces are arranged in the order indicated in Figs. 1 and 1<sup>bis</sup>, respectively, upon a recess fireproof table and then placed in the furnace in order to effect the welding together by producing a semi-fusion of the material under treatment. Fig.

2 illustrates the aspect which the blocks *a* and *b* of imitation material bear after having been welded upon the opposite faces of the plate *c*. The appearance is that of a block 55 in which the glass plate *c* separates the two blocks of imitation material *a* and *b*. Fig. 2<sup>bis</sup> illustrates the aspect which the block *a* of imitation material assumes after having been welded between the two pieces or plates 60 *c* and *c'*. Fig. 3 shows the aspect of the blocks *a* and *b* of differently-colored imitation materials after the welding upon one plate *c*.

The blocks thus produced irrespective of whether the masses or pieces of imitation material be colored or colorless are subsequently cut in the ordinary manner, but so that the parts of imitation material *a* and *b*, respectively, form one the top and the other the base, while the window-glass plate *c* forms 70 the crown.

When the blocks of imitation material *a* and *b* are colorless, the crown *c* of glass produces the following effect: As the plate *c* of glass is clearer and more transparent than the blocks *a* and *b* of imitation material, it, 75 causes the facets cut into the top and the base to more efficiently reflect and imparts to the stone thus formed scintillations and a fire similar to that of a real diamond. 80

When the blocks *a* and *b* of imitation substance are variously colored, the window-glass crown *c* produces the effect hereinafter indicated. First of all, seeing that the fusing-point of the glass is higher than that of the 85 imitation substance the window-glass plate *c* has not entered into combination with the blocks *a* and *b*, which have retained their proper color. Moreover, owing to the transparency of the window-glass the color of the 90 base will when the cutting has been effected appear all around the stone, without, however, penetrating to the top, where the color remains more intense and appears distinctly in the middle of the stone. 95

The cutting may of course be effected in any way and the number of facets does not in any manner modify the effect produced.

Fig. 3<sup>bis</sup> shows by way of modification a block of white or colored imitation material welded onto a plate or sheet *c* of window-glass. This modification is shown in section 100

and in perspective view. The block thus produced is subsequently cut in such a manner that the glass either forms the base, Fig. 4, or the top, Fig. 5. The result obtained in the case of this modification is identical with that before indicated.

It should finally be observed that in each one of the preceding examples the face or faces of the imitation substance in contact with the glass plate or plates may be polished prior to the welding operation.

I claim as my invention—

1. As a new article of manufacture, an artificial stone for use in jewelry, consisting of 15 clear transparent window-glass and "paste"

welded together into a single piece, substantially as described.

2. As a new article of manufacture, an artificial stone for use in jewelry, consisting of a top and bottom piece of "paste" and an intermediate layer of clear transparent window-glass welded together into a single piece, substantially as described.

In testimony whereof I have signed my name to this specification in the presence of 25 two subscribing witnesses.

SAMUEL GROSSIORD.

Witnesses:

THOS. N. BRONNE,  
MARIUS VICOY.